

April 8, 1947.

A. STERN

2,418,529

EMBRITTLED SILVER SOLDER BONDED ABRASIVE

Filed Dec. 4, 1944



Fig. 1



Fig. 2

Fig. 3

Inventor:  
Albert Stern  
By: Thues, Olson & Mucklow, burg  
Attest:

## UNITED STATES PATENT OFFICE

2,418,529

EMBRITTLED SILVER SOLDER BONDED  
ABRASIVE

Albert Stern, Chicago, Ill.

Application December 4, 1944, Serial No. 566,555

4 Claims. (Cl. 51—309)

1

My invention relates to a grinding wheel and more particularly to one utilizing diamond for its cutting action.

In grinding wheels the cutting action of the abrasive particles is at peak efficiency only when each particle may present unencumbered cutting edges to the material being worked upon. One of the principal drawbacks in the use of abrasive wheels is termed "glazing," caused by particles of material removed from the work embedding themselves in the spaces intermediate the cutting particles and thus interfering with the free action of the cutting edges. When glazing occurs it will rapidly build up to a stage where the wheel must be redressed to expose a fresh surface of abrasive to the work. Not only is this wasteful because of the discarded abrasive removed by the dressing operation but the work must be discontinued until dressing has been accomplished. Thus, useful production time is sacrificed. Furthermore, in the case of diamond wheels dressing is a slow and difficult operation.

Many attempts have been made to overcome glazing and eliminate redressing but without success, as the material thus far used to bond the wheel is generally of the same degree of plasticity and hardness as the particles of metal removed from the work and the bonding agent and the particles therefore conglomerate into a homogeneous mass where the original intention was that the particles of metal should embed themselves in the bonding agent and leave uninterrupted abrasive cutting particles projecting from the surface of the wheel.

I have found that a non-glazing wheel may be constructed in which the matrix comprises the principal abrasive ingredient, for example, diamond, together with another abrasive ingredient, for example, silicon carbide, and a bonding and filling agent including flakelets of mica and silver solder. While the theory of operation of my wheel is not thus far fully understood, one theory of operation seems to be that the mica and silver solder together form a sufficiently dense and tenacious bonding agent while being subject to easy attrition as the wheel wears in use. This may be due in part to the flaky nature of mica which imparts a lubricating quality permitting superimposed flakelets to slide one upon the other and be severed from the mass. Thus, as grinding proceeds, the particles of metal removed by the wheel will dislodge the flakelets and the silver solder dispersed between the abrasive particles and continuously allow a freshly exposed

2

series of cutting edges of the abrasive proper to be presented to the work.

Accordingly, the principal object of my invention is to provide a non-glazing grinding wheel in which the abrasive particles including one or more cutting materials are embedded in a matrix including comminuted mica and silver solder.

5 An additional object of my invention is to provide a non-glazing grinding wheel in which the matrix is of such character as to provide cleavage planes in the bonding agent.

10 Still another object is to provide a non-glazing grinding wheel including material subject to easy cleavage combined with material serving as a bonding agent for the abrasive particles.

15 Other objects are to provide a grinding wheel which will enable dry grinding to be done without glazing and to decrease the time of a grinding operation.

20 A further object of the invention is to provide a grinding wheel which is cooler in operation.

Another object is to enable the production of wheels of various grades by variation in the proportion of mica content.

25 An additional object is to provide a wheel including mica as part of the matrix whereby the latter is less brittle and hence not easily subject to breakage in use.

Other objects will appear as the description 30 proceeds.

In the drawings:

Fig. 1 is substantially a diagrammatic view of an apparatus in which the grinding wheel of the invention may be fabricated;

35 Fig. 2 is a diametrical cross section of a grinding wheel of the cup type embodying a grinding portion in accordance with my invention;

40 Fig. 3 is a magnified view through a portion of the work and a portion of the wheel, the cross section being taken to show the relative movement between the abrasive surface and the work; and

45 Fig. 4 is a fragmental portion of Fig. 3 on an even greater enlarged scale intended to show the theory of operation of my new wheel.

Referring first to Fig. 1, there is a hollow cylindrical molding chamber 9 in the aperture 10 of which is deposited a series of wheel blanks 11 cylindrical in form and including a plurality of 50 concentric keying grooves 12 adjacent the outer periphery of one flat face 13 thereof. Adjacent the face 13 of each blank 11 is a molding element 14 having a peripheral recess 15 of cross section to correspond with the contour of the grinding surface to be produced, i. e., rectangu-

lar, semi-circular, etc. Each of the blanks 11 and units 14 is pierced with a substantially central aperture 16, all in alignment.

In loading the chamber 9 there is first placed on the bottom a mass of a suitable fusible or thermoplastic bonding agent 20, e. g., silver solder, then a molding element 14 with its recess 15 uppermost. In the recess is substantially uniformly distributed material comprising a mixed predetermined quantity 21 of principal abrasive particles, e. g., diamond of a mesh suitable for the work to be performed by the wheel and of substantially uniform mesh, comminuted abrasive material of a hardness less than diamond, for example, silicon carbide, available commercially in one form under the trade name "Carborundum," and preferably of finer mesh than the principal particles, and comminuted mica which, due to the nature of the material, will be yielded as minute flakelets. A sufficient quantity of this mixture is distributed loosely into and piled slightly over the recess 15, the quantity being measured in advance and determined upon empirically. After the mixture 21 is thus deposited a wheel blank 11 is set into place as shown. Then another complete unit comprising an element 14, a mass of the mixture 21, and a wheel blank 11 is set in position, and so on, there being as many sets as is permitted by the capacity of the molding machine.

The entire molding unit is encased in a shield 22 extending upwardly into a hood 23 having a vent opening 24. Through apertures in the sides of the enclosure 22 extend a plurality of heating jets 25, only two being shown for clarity. Illuminating gas or any other suitable combustible fluid may be admitted to the jets 25 and ignited so that the flames play upon the outer surface of the chamber 9. The contents of the chamber, including the bonding agent 20 will be raised in temperature and when the agent reaches flowing temperature a piston 26 at the lower end of a screw 27 and fitting the aperture 10 is brought down upon the contents of the chamber, the pressure being sufficient to displace the melted mass of agent 20 upwardly through the central openings 16 and then radially outwardly in the spaces 28 intermediate each blank 11 and element 14 and into the interstices of the mixture 21. The pressure is applied gradually and the agent sustained in melted condition until the gaps 28 are entirely closed. When this occurs the mass of abrasive material, bonding agent and mica has been pressed into a homogeneous solid mass of the desired dimensions. Part of this mass enters the grooves 12 which serve to lock the annular abrasive portion proper of the wheel firmly to the wheel blank 11. Piston 26 is retracted, the chamber 9 allowed to cool, and the several complete wheel units may then be withdrawn.

The wheel units may be used in disc-like form as shown in Fig. 1 or may be turned on a lathe to any other desired shape, for example, cupped, as shown in Fig. 2.

Referring to Fig. 3, it will be noted that the matrix 20 will include the principal abrasive particles 31, e. g., diamond, sometimes commercially known as "bort," the subsidiary abrasive particles 32, e. g., silicon carbide, of smaller mesh, the mica flakelets 33, and the bonding agent 34, e. g., silver solder. Although I do not desire to limit myself herein to a matrix comprising any specified proportions of ingredients, I have found that a successful composition for most purposes will comprise 33 1/3% bort, 33 1/3% silicon carbide

in comminuted form and of a mesh finer than the bort, and 33 1/3% of mica flakelets of a mesh finer than the bort. The silver solder or other bonding agent which bonds the entire matrix is not to be considered a part of the proportions of the mix but only as a bonding agent. It will be understood that the size of the recess 15 and of the gap 28 may be so designed with respect to the amount of abrasive and the mica that only sufficient bonding agent to effect a thorough bond will be permitted to flow for formation of a matrix of the desired proportions.

In operation the particles of diamond will perform the major part of the grinding operation and these will be assisted by the particles of silicon carbide. However, it is intended that the latter named particles shall have a glaze-preventing action. That is, as attrition of the wheel occurs the particles of silicon carbide will be permitted to move within the mass to permit breaking down of the bonding agent and to assist in the movement of the mica flakelets. Otherwise stated, the action is intended to be similar to that occurring in a ball mill.

The mica flakelets, at least according to my theory of operation, tend to separate the bonding agent into disconnected strata. Hence, as attrition occurs those particles of silver solder near the surface slide freely on the mica flakelets and on each other and are carried away, either by the air stream in dry grinding or the lubricant in wet grinding, thereby leaving a constantly exposed cutting surface of diamond.

In Fig. 4, the reference numeral 35 indicates a high spot of the work which the grinding operation is intended to remove and it is shown midway between two diamond particles 31 and 31a. It is intended that a particular diamond particle 31a shall be the next to perform the cutting operation and it will be noted that the high spot 35 is engaged in gouging out the matrix shielding the cutting edge of the particle 31a so that the latter may present a properly exposed edge when it reaches the portion 35.

It will be comprehended that the invention is not limited to a diamond wheel but is capable of being embodied in any type of wheel, for example, one including silicon carbide alone as the abrasive agent. The gist of the invention resides in the inclusion of the mica flakelets with the matrix, and by "mica" I refer to any of those minerals commonly sold under the name "mica," there being several technically different types found in nature. However, they are all characterized by forming flakelets when comminuted, the natural planes of cleavage of mica yielding thin planiform particles or wafers having distinctive lubricating qualities when in such form.

One important advantage in the use of mica for the purpose outlined is its extreme resistance to disintegration under heat. Thus, although the wheel may reach a high temperature in operation, the mica flakelets will not break down into a form not possessing the desired characteristics outlined hereinabove. Notwithstanding the fact that the wheel may reach relatively high temperatures in operation during dry grinding, it is substantially cooler when wet grinding is being done. By reason of the fact that the mica is friable, pores are created in the matrix as grinding proceeds. These pores impart a spongy characteristic to the wheel enabling it to absorb substantial quantities of water and to cool the wheel.

Since the mica is a material relatively softer

than the other ingredients of the wheel, it is possible, by varying the proportion of mica, to construct wheels of varying degrees of hardness. Such gradation in the so-called "hardness" of the wheel renders the same exactly suited to the type of work being done. Metal bonded diamond wheels now known to the art are incapable of being so controlled in hardness.

Inasmuch as the wheel of my invention is, generally speaking, softer than other diamond wheels, it is not as subject to breakage, the matrix being more fibrous in nature as contrasted with the brittle construction of wheels presently known.

Trial has shown that the improved wheel of my invention is capable of increasing production as much as 30% over similar wheels not incorporating my improved matrix and that this increase is due to the non-glazing characteristic thus achieved.

Although I have shown by way of illustration the invention embodied in a grinding wheel, it will be comprehended that the abrasive composition is capable of use in other forms, for example, a whetstone.

Further modifications will be apparent to those skilled in the art and it is desired, therefore, that the invention be limited only by the scope of the appended claims.

Having thus described my invention, what I claim and desire to secure by Letters Patent is:

1. A substantially non-glazing abrasive body comprising a bonding matrix of silver solder having embedded therein substantial quantities of

abrasive particles and a filling agent consisting of mica-flakelets.

5 2. A substantially non-glazing abrasive body comprising a bonding matrix of silver solder having embedded therein substantial quantities each of diamond particles of substantially uniform size and silicon carbide and mica particles that are both smaller in size than said diamond particles.

10 3. A substantially non-glazing abrasive body comprising a silver solder bonding matrix having embedded therein substantial quantities each of abrasive particles of substantially uniform size and mica particles that are smaller in size than said abrasive particles.

15 4. A substantially non-glazing abrasive body comprising a bonding matrix of silver solder having embedded therein about equal parts each of silicon carbide particles of substantially uniform size and mica particles that are smaller in size than said silicon carbide particles.

ALBERT STERN.

#### REFERENCES CITED

25 The following references are of record in the file of this patent:

#### UNITED STATES PATENTS

| 30 | Number    | Name              | Date          |
|----|-----------|-------------------|---------------|
|    | 1,907,088 | Novotny           | May 2, 1933   |
|    | 2,197,655 | Boyer             | Apr. 16, 1940 |
|    | 2,223,063 | Fitz-Randolph     | Nov. 26, 1940 |
|    | 2,306,423 | Bernstorff et al. | Dec. 29, 1942 |